

## UNITED STATES PATENT OFFICE

2,450,888

## WEAR RESISTANT STEEL

Maurice C. Fetzer and Carl B. Post, Wyomissing,  
Pa., assignors to The Carpenter Steel Company,  
Reading, Pa., a corporation of New Jersey

No Drawing. Application July 27, 1946,  
Serial No. 686,725

4 Claims. (Cl. 75—123)

1

This invention relates to alloy steels, more particularly alloy steels containing not less than about 70 per cent by weight of iron and having a certain range of carbon content and being hardenable by quenching from above the critical temperature to a Rockwell C hardness of not less than about 53.

Those skilled in the art know that there are a considerable number of classes or types of alloy steels of the stated character such as hot work 10 steels, air hardening steels, shock resisting steels, hardenable stainless steels, and many others. Within each class, there are numerous specifically different compositions so that the total number of specifically different compositions is quite large.

The properties of the various classes and of the numerous species within the several classes differ depending on the number, kind and amount of alloying elements and the proportion of carbon. The various alloying elements include manganese, molybdenum, nickel, chromium, vanadium, tungsten, silicon and others. Properties such as hot and cold workability, tensile strength, impact strength, corrosion resistance, high temperature hardness and various other valuable properties are obtainable. Those skilled in the metallurgical art are fully informed regarding the composition of the numerous classes and species and the properties of alloy steels having those compositions.

With plain carbon steels, high abrasion resistance can be obtained by the use of tungsten but that expedient can not be satisfactorily employed in the case of most alloy steels and there has long been a need for means whereby the abrasion resistance of alloy steels in general can be markedly improved while maintaining intact the other valuable properties of the base.

It is the principal object of the invention to supply that long-felt want.

In accordance with the invention, the alloy steel base contains from about 0.3 to about 1.50 per cent by weight of carbon and is hardenable to an R. C hardness of not less than about 53. With that base, there is incorporated, for any particular carbon content within the range stat-

ed, a proportion of columbium carbide according to the following table.

2

| Percent Carbon in excess of carbon combined as Columbium Carbide | Percent Columbium Carbide to be added |           |
|------------------------------------------------------------------|---------------------------------------|-----------|
|                                                                  | Minimum                               | Maximum   |
| 0.30                                                             | About 3.6                             | About 4.5 |
| 0.40                                                             | About 3.4                             | About 4.0 |
| 0.50                                                             | About 3.1                             | About 3.6 |
| 0.60                                                             | About 2.7                             | About 3.3 |
| 0.70                                                             | About 2.6                             | About 3.1 |
| 0.80                                                             | About 2.4                             | About 2.9 |
| 0.90                                                             | About 2.2                             | About 2.7 |
| 1.00                                                             | About 2.0                             | About 2.5 |
| 1.10                                                             | About 1.8                             | About 2.4 |
| 1.20                                                             | About 1.7                             | About 2.3 |
| 1.30                                                             | About 1.6                             | About 2.2 |
| 1.40                                                             | About 1.5                             | About 2.1 |
| 1.50                                                             | About 1.5                             | About 2.0 |

The columbium carbide is incorporated by adding carbon and columbium in the ratio of about 1 part by weight of carbon to about 10 parts by weight of columbium, to form the per cent of columbium carbide desired.

For any content of carbon in the base between the limits of about 0.30 per cent by weight to about 1.50 per cent by weight, the approximate minimum proportion of columbium carbide must be added to obtain the improvement in wear resistance. The maximum stated should not be exceeded to avoid disturbing other valuable properties including transverse strength, impact strength, and ductility at room and elevated temperatures.

The carbon in the base alloy, as distinguished from carbon combined as columbium carbide, may be designated as matrix carbon. The advantages of the invention are not attainable by the use of matrix carbon without columbium carbide nor by the use of any or all proportions of matrix carbon and columbium carbide, but only by the conjoint use of certain restricted ranges of columbium carbide for a particular matrix carbon content, according to the table of correlated values above set forth.

The invention will be further described by reference to specific examples after first describing a test which has been found invaluable in measuring the wear resistance of steels.

The steels are machined into cylindrical specimens,  $\frac{3}{8}$ " dia. x 1" long, heat treated and then ground on both ends. One end of the specimen is held by firm pressure of about 5 lbs. against 5 120 grit alundum abrasive cloth, rotating at 1800 R. P. M. for six intervals of 5 seconds each. After each interval the specimen is cooled in water. The amount of metal ground away due to the 30 seconds of wear is measured with a vernier micrometer to the nearest .0001" ("tenth"). A new abrasive cloth is used for each specimen but not for each time interval. By exceptional wear is meant wear of not more than about one half that of the steel base, which is equivalent to stating that the improvement is about two fold and generally considerably more. For example, with a low carbon base (0.3 to 0.5% C) a wear of not exceeding about 80 "tenths" of an inch, whereas with a high carbon base (0.50 to 1.50% C) a wear of not exceeding about 40 "tenths" of an inch, may be obtained as measured by the above test.

#### Example 1

To a hot work steel containing 0.30 to 0.40% C, 3.5% Cr, 9.0% W, 25% V, and the balance substantially iron, there was added 2.75 to 5.50% of columbium carbide. These steels were cast into 2" sq. ingots, hammered to  $\frac{3}{8}$ " sq., and annealed. The wear specimens were then heated to 2175° F., oil quenched and tested as hardened and as drawn to 1050° F. The wear results follow:

| Ingot No. | Per Cent Matrix Carbon | Per Cent Columbium Carbide | As Oil Quenched, Wear in Tenths | As Oil Quenched, R. C | As Drawn, Wear in Tenths | As Drawn, R. C |
|-----------|------------------------|----------------------------|---------------------------------|-----------------------|--------------------------|----------------|
| X42379    | .36                    | 0                          | 200                             | 53                    | 110                      | 54             |
| 6322      | .35                    | 2.75                       | 141                             | 53                    | 118                      | 55             |
| 6323      | .37                    | 3.85                       | 40                              | 54                    | 20                       | 55             |
| 6324      | .38                    | 5.50                       | 31                              | 53                    | 12                       | 54             |

From the above data it is evident that the addition of about 3.8% columbium carbide to an alloy steel containing .30% C, 3.50% Cr, 9.0% W, 25% V, balance substantially iron, a high degree of abrasive wear resistance is obtained. Moreover, this high degree of abrasion resistance can be obtained without altering the other desirable properties of the steel base provided the per cent of columbium carbide is kept within the limits of the invention. That is illustrated by ingot 6324 which has good wear resistance but poor transverse ductility and other undesirable qualities. For a base containing about 0.30 to 0.40% carbon, the Cb C should not exceed about 4.0% to 4.50% by weight.

#### Example 2

To a hot work steel containing 0.35% C, 0.50% Mn, 1.0% Si, 5.0% Cr, 1.3% W, 1.4% Mo, .20% V, balance substantially iron, there were added various amounts of columbium carbide up to 4.5% columbium carbide. The two inch square ingots were hammered into bars,  $\frac{1}{8}$ " sq., annealed, machined into wear test specimens, hardened from 1850° F. in oil, tested and then drawn

at 950° F. and again tested. Results are as follows:

| Heat No. | Per Cent Matrix Carbon | Per Cent Columbium Carbide | Oil Treated, 1850° F., Wear in Tenths | Oil Treated, 1850° F., R. C. | As Drawn, Wear in Tenths | As Drawn, R. C. |
|----------|------------------------|----------------------------|---------------------------------------|------------------------------|--------------------------|-----------------|
| X64287   | 0.38                   | 0                          | 150                                   | 59                           | 150                      | 56              |
| 7361     | .41                    | 2.67                       | 113                                   | 60                           | 94                       | 58              |
| 7362     | .39                    | 3.24                       | 81                                    | 60                           | 86                       | 58              |
| 7363     | .41                    | 3.94                       | 38                                    | 59                           | 31                       | 58              |

From the above data it is evident that exceptionally good wear resistance is obtained on a 0.40% carbon hot work steel of the type described by the addition of approximately 4.0% columbium carbide. Columbium carbide additions in amounts greater than about 4.00 per cent cause low transverse ductility and other undesirable properties:

#### Example 3

This example relates to an air hardening base containing 2.00 to 3.00% manganese, 1.00 to 2.00% chromium, 1.00 to 2.00% molybdenum, 0.90 to 1.20% carbon and the balance substantially iron.

To a specific analysis of the above type steel containing initially about 1.00% C, columbium and carbon were added in proportions to provide about 1.1, 2.2 and 3.3% columbium carbide respectively. These steels were cast into  $1\frac{1}{2}$ " sq. ingots, weighing about 3 lbs., following which they were annealed, machined into wear test specimens, hardened from the most suitable hardening temperature, and then tested. The wear in "tenths" is given in the following table:

| Ingot No. | Percent Carbon in Base | Percent Columbium Carbide | Wear in Tenths | R. C Hardness |
|-----------|------------------------|---------------------------|----------------|---------------|
| 58        | 1.03                   | 0                         | 113            | 64            |
| 72        | 1.02                   | 1.15                      | 112            | 64            |
| 81        | 1.02                   | 2.20                      | 32             | 64            |
| 87        | 0.98                   | 3.32                      | 20             | 64            |
| 102       |                        |                           |                |               |

In the above example, the minimum and maximum percentages of columbium carbide should be correlated with the carbon in the base as follows:

| Percent C in Base | Percent Columbium Carbide |
|-------------------|---------------------------|
| 0.90              | About 2.2 to about 2.7    |
| 1.05              | About 1.9 to about 2.4    |
| 1.20              | About 1.7 to about 2.3    |

While ingot 102 has good wear resistant properties, it has poor transverse ductility which increases hot working difficulties.

Other examples of the invention are as follows:

#### Example 4

The base represents a commercial shock-resisting steel having a typical analysis range as follows:

|    |                                  |
|----|----------------------------------|
| C  | About .40 to about .60 per cent  |
| Mn | About .25 to about .90 per cent  |
| Si | About .90 to about 2.10 per cent |
| Cr | About .15 to about .30 per cent  |
| Mo | About .30 to about 2.00 per cent |
| W  | About .20 to about .50 per cent  |
| V  | About .20 to about .35 per cent  |

with or without one or more of the following:

With the above, there is incorporated about 2.7 to about 4.0 per cent of columbium carbide correlated with the carbon in the base according to the invention.

*Example 5*

The base represents a shock resisting hot work steel having a typical analysis range as follows:

C-----About 0.40 to about 0.60 per cent  
Mn-----About 0.25 to about 0.90 per cent  
Si-----About 0.25 to about 1.50 per cent  
Cr-----About 0.50 to about 1.80 per cent  
W-----About 1.00 to about 3.00 per cent  
V-----About 0.20 to about 0.35 per cent  
balance substantially iron.

With the above, there is incorporated about 2.7 to about 4.0 per cent of columbium carbide correlated with the carbon in the base according to the invention.

*Example 6*

The base represents a commercial oil hardening non-deforming tool steel having a typical analysis range as follows:

C-----About .80 to about 1.20 per cent  
Mn-----About 1.00 to about 1.80 per cent  
Si-----About 0.15 to about 0.45 per cent  
Mo-----About nil to about 0.40 per cent  
with or without one or more of the following:  
Cr-----About .20 to about .90 per cent  
W-----About .40 to about .70 per cent  
V-----About .15 to about .25 per cent  
balance substantially iron.

With the above there is incorporated 1.7 to 2.9 per cent by weight of columbium carbide correlated with the carbon in the base in accordance with the invention.

*Example 7*

The base represents a commercial hot work steel having a typical analysis range as follows:

C-----About 0.30 to about 0.70  
Mn-----About 0.15 to about 0.50  
Si-----About 0.15 to about 1.50  
Cr-----About 1.25 to about 8.0  
V-----About 0.25 to about 1.0

The above analysis includes 1.3 to 15.0% of tungsten or 1.5 to 5.0% molybdenum, or both, balance substantially iron.

With the above, there is incorporated from about 2.6 to about 4.5 per cent by weight of columbium carbide correlated with the carbon in the base in accordance with the invention.

*Example 8*

The base represents a commercial hardenable stainless steel having a typical composition range as follows:

C-----About 0.30 to about 1.10 per cent  
Mn-----About 0.15 to about 0.50 per cent  
Si-----About 0.15 to about 0.50 per cent  
Cr-----About 12.5 to about 19.0 per cent  
with or without either or both of the following:

Mo-----About 0.25 to about 0.75 per cent  
V-----About 0.10 to about 0.30 per cent  
balance substantially iron.

With the above, there is incorporated from about 1.8 to about 4.5 per cent by weight of columbium carbide correlated with the carbon in the base in accordance with the invention.

*Example 9*

The base represents a commercial high carbon, high chromium tool steel having a typical composition range as follows:

5 C-----About 1.20 to about 2.40 per cent  
Mn-----About 0.10 to about 0.60 per cent  
Si-----About 0.15 to about 0.75 per cent  
Cr-----About 11.0 to about 13.5 per cent  
10 with or without one or more of the following:  
Mo-----About 0.60 to about 1.0 per cent  
Ni-----About 0.50 to about 1.0 per cent  
Co-----About 0.50 to about 3.0 per cent  
V-----About 0.15 to about 1.0 per cent  
15 balance substantially iron.

With the above, there is incorporated from about 1.5 to about 2.3 per cent of columbium carbide correlated with the carbon in the base  
20 in accordance with the invention.

*Example 10*

The base represents a commercial chromium nickel steel having a typical composition range as follows:

25 C-----About 0.40 to about 1.40 per cent  
Cr-----About 0.20 to about 1.50 per cent  
Ni-----About 1.0 to about 4.5 per cent  
30 with or without one or more of the following:  
W-----About 1.0 to about 2.5 per cent  
V-----About 0.10 to about 0.25 per cent  
balance substantially iron.

With the above, there is incorporated about 35 1.5 to about 4.0 per cent by weight of columbium carbide correlated with the carbon in the base in accordance with the invention.

*Example 11*

40 The base represents a ball and bearing steel having a typical composition range as follows:

C-----About 0.80 to about 1.10 per cent  
Mn-----About 0.20 to about 1.75 per cent  
Si-----About 0.15 to about 1.75 per cent  
Cr-----About 0.35 to about 3.0 per cent  
balance substantially iron.

With the above there is incorporated about 1.80 to about 2.90 per cent by weight of columbium carbide correlated with the carbon in the base  
50 in accordance with the invention.

*Example 12*

55 The base represents a commercial carbon vanadium water hardening tool steel having a typical composition range as follows:

C-----About 0.60 to about 1.25 per cent  
Mn-----About 0.15 to about 0.35 per cent  
Si-----About 0.15 to about 0.50 per cent  
V-----About 0.08 to about 0.40 per cent  
balance substantially iron.

With the above there is incorporated about 1.6 to about 3.3 per cent by weight of columbium carbide correlated with the carbon in the base in accordance with the invention.

*Example 13*

70 The base represents a commercial valve steel having a typical composition range as follows:

C-----About 0.30 to about 0.50 per cent  
Mn-----About 0.20 to about 1.0 per cent  
Si-----About 2.0 to about 4.0 per cent  
75 Cr-----About 7.0 to about 9.0 per cent

with or without one or more of the following:

Ni ----- About 0.50 to about 1.0 per cent  
 Mo ----- About 0.25 to about 1.0 per cent  
 W ----- About 1.0 to about 3.0 per cent  
 balance substantially iron.

With the above there is incorporated about 3.1 to about 4.5 per cent by weight of columbium carbide correlated with the carbon in the base in accordance with the invention.

This application is a continuation-in-part of application Serial No. 529,366, filed April 3, 1944, now abandoned.

What is claimed is:

1. The combination of about 1.5 to about 4.5 per cent by weight of columbium carbide, with an alloy steel base, said base containing not less than about 70 per cent by weight of iron, about 0.30 to about 1.50 per cent by weight of carbon and being hardenable by quenching to a Rockwell C hardness not less than about 53, the columbium carbide being composed of columbium and carbon in the weight ratio of about 10 to 1, and the minimum and maximum percentages by weight of columbium carbide being correlated with the per cent by weight of carbon in the hardenable base as follows:

| Per cent by weight of Columbium carbide |              | Per cent by weight of Carbon in the base |
|-----------------------------------------|--------------|------------------------------------------|
| Minimum                                 | Maximum      |                                          |
| About 3.6                               | to about 4.5 | About 0.30                               |
| About 3.4                               | to about 4.0 | About 0.40                               |
| About 3.1                               | to about 3.6 | About 0.50                               |
| About 2.7                               | to about 3.3 | About 0.60                               |
| About 2.6                               | to about 3.1 | About 0.70                               |
| About 2.4                               | to about 2.9 | About 0.80                               |
| About 2.2                               | to about 2.7 | About 0.90                               |
| About 2.0                               | to about 2.5 | About 1.00                               |
| About 1.8                               | to about 2.4 | About 1.10                               |
| About 1.7                               | to about 2.3 | About 1.20                               |
| About 1.6                               | to about 2.2 | About 1.30                               |
| About 1.5                               | to about 2.1 | About 1.40                               |
| About 1.5                               | to about 2.0 | About 1.50                               |

2. The combination of about 1.7 to about 2.7 per cent by weight of columbium carbide with an air hardening alloy steel base containing about 0.90 to about 1.20 per cent by weight of carbon and being hardenable by quenching to a Rockwell C hardness of not less than about 53, said base also containing about 2 to 3 per cent by weight of manganese, about 1 to 2 per cent by weight of chromium, and about 1 to 2 per cent by weight of molybdenum, balance substantially iron, the columbium carbide being composed of columbium and carbon in the weight ratio of about 10 to 1, and the minimum and maximum percentages by weight of columbium carbide being correlated with the per cent by weight of carbon in the base as follows:

| Per cent by weight of Columbium Carbide |              | Per cent by weight of Carbon in the Base |
|-----------------------------------------|--------------|------------------------------------------|
| Minimum                                 | Maximum      |                                          |
| About 2.2                               | to about 2.7 | About 0.9                                |
| About 2.0                               | to about 2.5 | About 1.0                                |
| About 1.8                               | to about 2.4 | About 1.1                                |
| About 1.7                               | to about 2.3 | About 1.2                                |

3. The combination of about 2.6 to about 4.5 per cent by weight of columbium carbide with a hardenable hot work alloy steel base containing about 0.30 to about 0.70 per cent by weight of

carbon and being hardenable by quenching to a Rockwell C hardness of not less than about 53, said base also containing about 0.15 to about 0.50 per cent by weight of manganese, about 0.15 to about 1.50 per cent by weight of silicon, about 1.25 to about 8.00 per cent by weight of chromium, about 0.25 to about 1.0 per cent by weight of vanadium, and an element selected from the group consisting of tungsten in the amount of about 1.3 to about 15.0 per cent by weight and molybdenum in the amount of about 1.5 to about 5.0 per cent by weight, balance substantially iron, the columbium carbide being composed of columbium and carbon in the weight ratio of about 10 to 1, and the minimum and maximum percentages by weight of columbium carbide being correlated with the per cent by weight of carbon in the base as follows:

| 20        | Per cent by weight of Columbium Carbide |         | Per cent by weight of Carbon in the Base |
|-----------|-----------------------------------------|---------|------------------------------------------|
|           | Minimum                                 | Maximum |                                          |
| About 3.6 | to about 4.5                            |         | About 0.30                               |
| About 3.4 | to about 4.0                            |         | About 0.40                               |
| About 3.1 | to about 3.6                            |         | About 0.50                               |
| About 2.7 | to about 3.3                            |         | About 0.60                               |
| About 2.6 | to about 3.1                            |         | About 0.70                               |
| About 2.4 | to about 2.9                            |         | About 0.80                               |
| About 2.2 | to about 2.7                            |         | About 0.90                               |
| About 2.0 | to about 2.5                            |         | About 1.00                               |
| About 1.8 | to about 2.4                            |         | About 1.10                               |
| About 1.7 | to about 2.3                            |         | About 1.20                               |
| About 1.6 | to about 2.2                            |         | About 1.30                               |
| About 1.5 | to about 2.1                            |         | About 1.40                               |
| About 1.5 | to about 2.0                            |         | About 1.50                               |

4. The combination of about 1.7 to about 2.9 per cent by weight of columbium carbide with a hardenable non-deforming oil-hardening alloy steel base containing about 0.80 to about 1.20 per cent by weight of carbon and being hardenable by quenching to a Rockwell C hardness not less than about 53, said base also containing about 1.00 to about 1.80 per cent by weight manganese, about 0.15 to about 0.45 per cent by weight silicon, about 0.15 to about 0.40 per cent by weight molybdenum, about 0.20 to about 0.90 per cent by weight chromium, about 0.40 to about 0.70 per cent by weight tungsten, and about 0.15 to about 0.25 per cent by weight vanadium, said chromium, tungsten and vanadium being optional, the columbium carbide being composed of columbium and carbon in the weight ratio of about 10 to 1, and the minimum and maximum percentages by weight of columbium carbide being correlated with the per cent by weight of carbon in the base as follows:

| 50        | Per cent by weight of Columbium Carbide |         | Per cent by weight of Carbon in the Base |
|-----------|-----------------------------------------|---------|------------------------------------------|
|           | Minimum                                 | Maximum |                                          |
| About 2.4 | to about 2.9                            |         | About 0.8                                |
| About 2.2 | to about 2.7                            |         | About 0.9                                |
| About 2.0 | to about 2.5                            |         | About 1.0                                |
| About 1.8 | to about 2.4                            |         | About 1.1                                |
| About 1.7 | to about 2.3                            |         | About 1.2                                |

MAURICE C. FETZER,  
 CARL E. POST.

#### REFERENCES CITED

The following references are of record in the file of this patent:

#### FOREIGN PATENTS

| Number  | Country       | Date          |
|---------|---------------|---------------|
| 457,760 | Great Britain | Nov. 30, 1936 |
| 507,983 | Great Britain | June 23, 1939 |